

## UNITED STATES PATENT OFFICE

1,938,608

## PROCESS OF PURIFYING METAL

William H. Osborn and Harry H. Stout, Jr., New York, N. Y., assignors to Coalescence Products Company, Inc., New York, N. Y., a corporation of New York

No Drawing. Application August 7, 1931  
Serial No. 555,858

6 Claims. (Cl. 148—16)

This invention relates to a process for removing impurities from metal particles.

My co-pending application Serial No. 299,665 now Patent No. 1,822,939, issued September 15,

5 1931 discloses a process for coalescing metals in which separate metal particles are coalesced into a solid homogeneous mass after the surfaces of the particles have been treated to remove impurities that would interfere with the coalescence.

10 The present invention has for its object an improved method of cleaning the metal particles preparatory to coalescence.

A particular object of the invention is to provide a mixture of gases, in the cleaning of the surfaces of copper particles of combined or adhering impurities, which is reducing to copper oxide but neutral or non-reducing to sulphur dioxide ( $\text{SO}_2$ ).

Another particular object is to provide a mixture of gases, in the cleaning of the surfaces of copper particles of combined or adhering impurities, which is reducing to copper oxide but oxidizing to carbon and carbonaceous material present on the surfaces of the copper particles.

25 The invention provides a safe and economical method for carrying out these objects.

The invention will be described in detail as applied to the cleaning of electrolytically deposited copper particles, although obviously the same principles can be applied to copper particles produced in other ways, or to particles of other metals, or alloys.

In the electrolytic refining of copper the cathode deposit is made in an electrolyte containing sulphuric acid ( $\text{H}_2\text{SO}_4$ ), copper sulphate ( $\text{CuSO}_4$ ) and other metallic salts as impurities.

In withdrawing the cathode from the electrolyte some of it adheres to the copper and leaves on drying some of these metallic salts and other 40 impurities entrained on the surfaces of the cathode crystals.

Much of these entrained impurities may be removed by washing the cathode in hot water or other solvents but within the limits of practical 45 operation it is not possible to do so completely.

Further, on exposure to the air, the surfaces of the cathode crystals become oxidized, the extent of the oxidation depending on length and conditions of exposure.

50 In using brittle cathodes made by depositing against a copper blank coated with an organic compound from which the deposit is stripped a further impurity results from carbonaceous material of the coating compound adhering to the cathode.

To recapitulate—The impurities found on copper cathode and to which this invention refers are—

1. Sulphur from entrained sulphate.
2. Oxygen from exposure to the air and present in the sulphates.
3. Carbonaceous material from the coating compound.

4. Arsenic and antimony from the electrolyte which is incidentally partially removed by the process.

In the coalescence of copper, temperature and pressure are so exerted on a mass of separate copper particles as to cause grain growth to occur across the original particle surfaces. In order that this grain growth shall not be retarded it is necessary that no film or surface of material (such as  $\text{Cu}_2\text{O}$ ,  $\text{Cu}_2\text{S}$ ,  $\text{CuSO}_4$ , etc.) other than pure copper be interposed between the surfaces of the copper particles. 75

Hence, in coalescing cathode material containing impurities as described above it is necessary at the temperatures at which coalescence takes place, and until coalescence is complete, that these impurities shall have been removed from the particle surfaces. 80

Our experimentation has disclosed in respect to the elimination of sulphur from cathode copper—

First.—That for the generalized equation for the dissociation of copper sulphate, viz:



which begins at approximately 650° F. and is complete below 1400° F., the  $\text{SO}_2$  gas formed is practically non-reactive to copper, i. e., the equation—



does not become active below 1600° F. and hence if copper and copper sulphate are heated in a current of any neutral carrier gas such as nitrogen to temperatures above the final dissociation point of  $\text{CuSO}_4$ , the  $\text{SO}_2$  formed is swept out by the current of neutral gas and the sulphur substantially eliminated from the copper. 95 100

Second.—That the reduction of sulphur dioxide ( $\text{SO}_2$ ) by hydrogen to S or  $\text{H}_2\text{S}$  according to the equations—



or



is very slight at 500° F. but becomes increasingly 110

active with increase of temperature and is marked above 1000° F.

For example, in passing a mixture of equal volumes of  $\text{SO}_2$  and  $\text{H}_2$  through an externally heated 5 glass tube at 500° F. no S was condensed in the cold portion of the tube, but above 1000° marked condensation of S was observed.

Placing deoxidized, desulphurized copper particles in the tube treated with the same mixture 10 of gases at 500° F. the copper particles on analysis showed 0.008% S, at 1000° F. 0.03% S and at 1500° F. 0.8% S.

In other words, as the temperature was increased more  $\text{SO}_2$  was reduced to elemental S by 15 the  $\text{H}_2$  and combined with the copper to form  $\text{Cu}_2\text{S}$ .

*Third.*—That the equation



20 being a reversible one the addition of excess steam to the gas mixtures prevented the formation of S as follows:

At 1000° F. the formation of S was completely stopped by addition of 50%  $\text{H}_2\text{O}$  vapor to the gas 25 mixture. At 1500° F. the addition of 90%  $\text{H}_2\text{O}$  vapor was insufficient to prevent formation of S. But by using a larger proportion of steam, having less than 1% of hydrogen present in the steam, the formation of S can be prevented below 1600° F.

30 *Fourth.*—That for the equilibrium equation—



35 at temperatures below 1600° F. the vapor pressure of  $\text{H}_2\text{S}$  formed is very slight and a great excess of  $\text{H}_2$  is required to desulphurize the copper. Hence, if in the presence of copper,  $\text{SO}_2$  is reduced by  $\text{H}_2$  to S and combines with the copper to form  $\text{Cu}_2\text{S}$  it requires a long time and much excess of  $\text{H}_2$  to finally eliminate all S.

40 *Fifth.*—That  $\text{Cu}_2\text{S}$  having been formed, water vapor ( $\text{H}_2\text{O}$ ) present in the current of  $\text{H}_2$  greatly accelerates removal of S. This is because by the equilibrium reaction:



45 some  $\text{SO}_2$  is formed and this being substantially unreactive to copper is swept out by the current of gas.

50 *Sixth.*—That carbon monoxide (CO) reduces  $\text{SO}_2$  to elemental S (for method see above with  $\text{H}_2 + \text{SO}_2$ ) but that the reaction is not active before reaching a temperature of 1100° F. and that at 1500° F. the presence of 85% water vapor 55 is sufficient to repress the reduction to S.

55 *Seventh.*—That the  $\text{SO}_2$  dissociated below the point where its reduction by  $\text{H}_2$  is very active is swept out by a current of  $\text{H}_2$  just as by any other carrier gas and that this effect may account for 60 the elimination of better than 60% of the original S present as sulphates during period of heating to 1600° F. The mixture of steam and hydrogen used in the preferred form of the present invention also acts to sweep away the  $\text{SO}_2$ .

65 Our experimentation has disclosed in respect to the elimination of oxygen from cathode copper—

70 *First.*—That both  $\text{H}_2$  and CO will completely deoxidize cathode material at temperatures above 1000° F. but that in passing a current of gas over the surface of oxidized particles the efficiency of reduction is much greater with CO than with  $\text{H}_2$ .

75 *Second.*—That pure steam ( $\text{H}_2\text{O}$ ) alone is

slightly oxidizing to copper at temperatures between 1000° F. and 1600° F.

*Third.*—That water vapor or oxygen present with  $\text{H}_2$  at temperatures above 1000° F. will not prevent reduction of copper oxide but that at 80 some point below 800° F. the reaction—



is no longer sufficiently active to prevent the reoxidation of the metal by traces of steam or 85 oxygen present.

Hence in determining the deoxidation of copper by a current of wet  $\text{H}_2$  at temperatures over 1000° F. it is necessary to cool in a current of a dry neutral gas such as  $\text{N}_2$  or else to reduce the 90 flow of  $\text{H}_2$  and then cool so quickly as to substantially prevent the secondary reoxidation which takes place at some point below 800° F.

*Fourth.*—That the equilibrium reaction between metallic iron and steam at temperatures between 1200° F. and 1600° F. yields  $\text{H}_2$  in a ratio of  $\text{H}_2$  to  $\text{H}_2\text{O}$  in excess of the amount of  $\text{H}_2$  required to be reducing to copper.

*Fifth.*—Investigation of known equilibrium reactions indicated that at 1650° F. only approximately one part  $\text{H}_2$  to 76,000 parts of steam was theoretically necessary to produce a gas mixture neutral to copper. Our experimentation has shown that one part  $\text{H}_2$  in approximately 1200 parts of  $\text{H}_2\text{O}$  at 1600° F. is sufficient to produce 105 a condition actually reducing to copper.

Our experimentation has disclosed in respect to the elimination of carbonaceous material adhering to the surfaces of copper particles—

*First.*—That by the well-known water gas reaction—



carbon and hydrocarbon residues are completely removed from the surfaces of copper particles.

*Second.*—That neither dry  $\text{H}_2$  nor CO would alone remove carbon.

*Third.*—That in treating brittle cathode which was briquetted or baled into billet shape the rate at which carbon residue was removed by 120 a current of steam varied inversely with the density of the briquetted billet. For example, a billet briquetted to 83% of the density of solid copper and containing asphalt residue from the embrittling agent to the extent of about .0025% 125 of the weight of the copper was treated for 35 minutes in a current of  $\text{H}_2\text{O}$  above 1000° F. up to 1600° F. and showed complete elimination of carbon residue. A billet briquetted to 92% of the density of solid copper and treated in the 130 same manner required one hour at 1600° F. to effect complete elimination of carbon.

In summarizing our experimentation we found—

*First.*—That as little as one part hydrogen in 135 1200 parts water vapor was at temperatures above 1200° F. reducing to copper oxide.

*Second.*—That  $\text{SO}_2$  gas produced by dissociation of metallic sulphates substantially did not affect copper at the temperatures studied but 140 that it reduced to S or  $\text{H}_2\text{S}$  by  $\text{H}_2$  or CO, the S formed did combine with copper to form  $\text{Cu}_2\text{S}$  and was then hard to remove.

*Third.*—That a sufficient excess of steam prevented the reduction of  $\text{SO}_2$  to S by either  $\text{H}_2$  145 or CO.

*Fourth.*—That steam was an efficient remover of carbon adhering to the copper particle surfaces.

By combining the results of this experimenta-

tion so as to provide most efficiently for removal of dissociated  $\text{SO}_2$ , for reduction of oxygen and for elimination of carbon, we found that by treating cathode particles containing slight amounts of hydrocarbon residues in a current of steam containing less than 1% by volume of  $\text{H}_2$  at elevated temperatures up to  $1600^{\circ}\text{ F.}$ , substantially complete elimination of  $\text{O}_2$ ,  $\text{S}$  and  $\text{C}$  were obtained in less than one hour's treatment above  $1000^{\circ}\text{ F.}$  This result is due to the fact that this combination of steam and hydrogen is:

- (a) Reducing to oxides of copper.
- (b) Neutral to  $\text{SO}_2$ .
- (c) Oxidizing to C.

We found that in the case of copper particles briquetted to too great density the reaction between steam and carbon produced within the billet a local concentration of reducing gases sufficiently high to reduce  $\text{SO}_2$  present and hinder the complete elimination of  $\text{S}$ , but that if the density of the billet did not exceed approximately 83% of that of solid copper and if the amount of carbon present was kept to a minimum, the local reducing condition was not sufficient to reduce  $\text{SO}_2$  and substantial removal of  $\text{S}$  was obtained.

In applying the process to other forms of copper, for example shotted copper, it is preferred to alter the composition of the cleaning gas, increasing the percentage of hydrogen to 10 or 15%. Changes in the percentages of hydrogen and steam may also be made in applying the process to other metals, such as nickel.

We claim:

1. The process of purifying metallic particles which comprises treating the metallic particles at an elevated temperature below the melt point of the metallic particles with a gaseous mixture

comprising approximately 85% steam and 15% hydrogen, by volume.

2. The process of purifying metallic particles which comprises treating the metallic particles at an elevated temperature below the melt point of the metallic particles with a gaseous mixture comprising approximately 99% steam and 1% hydrogen, by volume. 86

3. The process of purifying copper which comprises treating copper at an elevated temperature below the melt point of copper with a gaseous mixture comprising approximately 85% steam and 15% hydrogen, by volume. 85

4. The process of purifying copper which comprises treating copper at an elevated temperature below the melt point of copper with a gaseous mixture comprising approximately 99% steam and 1% hydrogen, by volume. 90

5. The process of purifying metallic particles which comprises treating the metallic particles at an elevated temperature below the melt point of the metallic particles with a gaseous mixture which is reducing to the oxides of the metallic particles, oxidizing to carbon, and neutral to sulphur dioxide, said gaseous mixture consisting of from less than 1% by volume to 15% by volume of hydrogen, the remainder being steam. 95

6. The process of purifying metallic particles which comprises treating the metallic particles at an elevated temperature below the melt point of the metallic particles with a gaseous mixture which is reducing to the oxides of the metallic particles, oxidizing to carbon, and neutral to sulphur dioxide, said gaseous mixture consisting of from 85 to 99% by volume of steam and from 15 to 1% by volume of hydrogen. 105 113

WILLIAM H. OSBORN.  
HARRY H. STOUT, JR.

40

115

45

120

50

125

55

130

60

135

65

140

70

145

75

150